

Dec. 5, 1939.

O. E. HARDER

2,182,758

STEEL

Filed May 14, 1938



*Fig. 1*



*Fig. 2*



*Fig. 3*

INVENTOR  
Oscar E Harder

BY

*Corbett & Mahoney*  
ATTORNEYS

## UNITED STATES PATENT OFFICE

2,182,758

## STEEL

Oscar E. Harder, Columbus, Ohio, assignor to In-  
land Steel Company, Chicago, Ill., a corpora-  
tion of Delaware

Application May 14, 1938, Serial No. 208,069

9 Claims. (CL. 75—123)

This invention relates to steel. It has to do particularly with those types of steel which are likely to be subjected to machining operations before being ultimately placed in use, although it is not necessarily limited thereto.

In the prior art, the practice most generally resorted to for the purpose of improving the machinability of steel is the addition of sulfur to the steel. Sometimes, selenium is used, though the cost thereof is somewhat prohibitive. Normally, where sulfur or selenium are used for improving the machinability of the steel, they are introduced in such quantities as to insure a recovery in the steel of more than .05 per cent sulfur or selenium, or if both are used a total in excess of .05 per cent is usually required.

For example, certain "free cutting" steels have attained a well established and recognized classification in the steel industry. The Society of Automotive Engineers recognizes this special class of steel and has provided standard specifications for their chemical composition.

These steels are all characterized by higher sulfur contents (.075—0.300 per cent) than is common in steels which do not fall within the class of free cutting steels. It can probably be said that thus increasing the sulfur content is the commonly accepted method of improving the machinability of steels and bringing them within the class of free cutting steels.

However, the use of sulfur in such relatively high percentages for the purpose of improving the machinability of the steels has certain important drawbacks and limitations. It has a tendency to cause trouble in hot-working the steel, as in rolling the ingot. Therefore, it is common practice to hot-work these free cutting steels containing relatively high sulfur contents at higher temperatures than with steels of lower sulfur contents. Also, it is general metallurgical practice to use relatively high percentages of manganese when the sulfur content is increased in order to avoid or minimize hot shortness in the steel, that is, to avoid brittleness or lack of strength of the steel at red heat. In addition, the use of too much sulfur in steel has a tendency to impart thereto objectionable physical properties, such as low ductility.

It is also recognized that, under some conditions, increased phosphorus content tends to improve the machinability of steels. This is especially true with steels which are low in carbon content and which are relatively soft and tend to "drag" during the machining operation. It is recognized that increasing the phosphorus content may serve to overcome this drawback. However, there are limitations to the improvement of

the machinability of steels by increasing the phosphorus content. Too much phosphorus may give undue hardness and detract from the desired ductility. In certain classes of steels a certain amount of ductility is necessary and the use of increased phosphorus contents for the purpose of producing a free cutting steel is impracticable because of its tendency to decrease ductility.

Bessemer steels normally make better free cutting steels than open-hearth steels. However, Bessemer steels are now somewhat more costly to produce and more difficult to control as to composition than open-hearth steels and some steel plants do not have Bessemer furnaces. Because of these and other reasons, the demand for open-hearth steels, during recent years, has been increasing at the expense of the demand for Bessemer steels. Therefore, it would be highly desirable to produce open-hearth steels having as good machinability as Bessemer steels. Nevertheless, it has not been possible to accomplish this by increasing the sulfur content without harmfully sacrificing important physical properties.

While considerable progress has been made in improving the machinability of steel, mainly by increasing the sulfur content, and while the industry now has at least nine steels which are listed in S. A. E. specifications, so that selections can be made from these types in accordance with the required machinability and the desired mechanical properties in the finished product, there still remains a need to further improve the free cutting characteristics of steel. This is especially true if such improvement can be attained without loss of other desirable characteristics, such as good hot working properties and adequate ductility and other physical properties. It is known that investigators have conducted extensive researches directed to the improvement of free cutting steels in which they have varied the chemical compositions and have studied new methods of adding such elements as sulfur, phosphorus, manganese and carbon, and have varied the amount of retained oxygen in the steel.

However, there has been no marked improvement over the prior art until the present invention. This invention rests primarily in the fact that it has been discovered that the machinability of steels can be improved by the incorporation of lead in the steel, provided the lead is introduced under such conditions and in such a way as to insure that there will be retained in the steel, upon solidification, an adequate quantity of the lead existing in the steel in a state of dispersion. Thus, a "free cutting" steel can be produced by incorporation of the lead in the steel either as a substitute for part or substan-

tially all of the sulfur commonly used in the so-called "free cutting" steels or as a supplement for such sulfur, provided the lead is added in such quantities and under such conditions as to insure a comparatively uniform dispersion of the lead throughout the steel. It has also been found that lead thus incorporated in the steel will improve the machinability thereof, even though it does not result in the production of a steel that would be classified as a "free cutting" steel. Likewise, it has been found that the lead so incorporated does not materially reduce the desirable mechanical properties of the steel. The novelty of this discovery is accentuated by the fact that many investigators have studied the alloys of iron and lead and of steel and lead and have reported in the technical literature that lead is insoluble in iron. These reports have undoubtedly deterred other investigators from the use of lead as an addition agent to steel for the purpose of improving the machinability and, particularly, for the making of free cutting steel.

Dr. M. Hansen in his book on binary alloys published by Julius Springer, Berlin, in 1936, on page 716, reviews the information on iron-lead alloys. His diagrams show no solubility below the melting point of iron and above that temperature there are two liquid layers with only very slight solubility. He quotes Isaac and Tammann (Z. Anorg. Allg. Chem., vol. 55 (1907), page 58) who concluded that the metals are practically insoluble in each other in the liquid state. Hansen also quotes Stevenhagen and Schucard (Z. Anorg. Allg. Chem., vol. 186 (1930), page 277) that the solidified product forms in sharp layers and the metals are practically insoluble in each other. He quotes from Tammann and Oelsen (Ber. Itsch Chem. Ges., vol. 35 (1902), page 910), that the solubility of iron in lead is  $3 \times 10^{-4}$  per cent and that lead has no influence on the transformation temperatures of iron. Undoubtedly, the researches which have been reported in the literature, as exemplified by the above, have deterred other investigators from the use of lead as an addition agent to steel for the purpose of improving the machinability and, particularly, for the making of free cutting steels.

I am aware of the fact that certain prior art patentees have suggested the use of lead in ferrous metals but such suggestions have either contemplated the use of lead in cast iron or special alloy steel or have been based more or less on the general idea that the lead would either purify or alter the nature of the steel in such a manner as to minimize the occurrence of defects in the ingots formed therefrom. In some cases, the amounts of lead proposed have been so large as to show a complete lack of understanding of the practical aspects of steel making and marketing. At any rate, no patent with which I am familiar, has taught the art, or even suggested that the introduction of lead into normal steels could be made effective to improve the machinability thereof, nor has any prior investigator or patentee ever suggested that lead, when introduced into steel in proper percentages would be effective to render the steel "free cutting" either alone or in combination with sulfur or any other element.

This application is a continuation in part of my application, S. N. 177,292, filed November 30, 1937.

In the pursuance of my development, lead has been added to the steel by a number of methods

which will be discussed more in detail herein-after. At this point, it will suffice to say that it seems to be important that the lead be added to the steel in subdivided form and under conditions wherein considerable agitation of the steel is occurring. For example, lead has been successfully dispersed throughout the steel by introducing it into molten steel in a crucible in a high frequency induction furnace which naturally causes an agitation of the steel. It has also been successfully dispersed throughout the steel by introducing it into ingot molds during the pouring operation and preferably starting the introduction of lead early in the filling of the mold. It is also important that the lead be introduced in quantities sufficient to insure that the amount desired is retained in the steel. For example, my tests show that the introduction of lead in percentages approximating 1 per cent by weight of the steel may result in a recovery of about .50 to .70 per cent lead under favorable conditions.

Lead-containing steels, made in accordance with my invention, have certain characteristic microstructures which can be brought out by metallographic technique and these structures are characteristic of these lead-bearing steels of improved machinability.

Duplications of photomicrographs, at a magnification of 500 diameters, are shown in the accompanying drawing and a comparison of the microstructure shown therein will make this relation clear.

Figure 1 represents a photomicrograph of steel A which is so designated in Table I, immediately following, which table sets forth the constituents of this steel and shows that it contains no lead.

Figure 2 shows the microstructure of steel B which is also included in Table I, immediately following, which table shows that the steel has practically the same chemical composition as steel A, except that it contains 0.12 per cent of lead in addition to its other constituents.

Figure 3 shows the microstructure of steel C which is so designated in Table I, immediately following, which table sets forth the constituents of this steel and shows that it has practically the same chemical composition as steel A, except that it contains 0.478 per cent of lead.

The Table I referred to is as follows:

TABLE I.—Chemical composition of steels A, B and C

| Steel No. | Chemical composition—percent |       |      |       |       |       |
|-----------|------------------------------|-------|------|-------|-------|-------|
|           | C                            | Si    | Mn   | S     | P     | Pb    |
| A-----    | 0.11                         | 0.012 | 0.63 | 0.193 | 0.017 | None  |
| B-----    | 0.10                         | 0.012 | 0.55 | 0.204 | 0.019 | 0.12  |
| C-----    | 0.11                         | 0.008 | 0.62 | 0.235 | 0.017 | 0.478 |

The lead is apparently dispersed throughout the steel partly in sub-microscopic form. The multiplicity of small black spots, which are stains made apparent by the etching process and which are so prevalent in the lead-containing steels of Figures 2 and 3 in comparison with the substantial absence thereof in the steel of Figure 1 which contains no lead, clearly indicates that the lead is fully dispersed throughout the steel. Electrical conductivity tests which I have made show that resistivity is not increased by the lead and this suggests that the lead is not in solid solu-

tion in the steel but is present in a dispersed form.

I have added lead to molten steels of essentially the same compositions as steel A in different amounts as the mineral galena (PbS with approximately 86.6 per cent Pb and 13.4 per cent S) to produce steels B and C. Many other steels containing lead have been made and studied using experimental heats ranging from 15 to 300 pounds and commercial ingots weighing of the order of 11,000 pounds.

While the lead in steels B and C was added as galena, it has been found that the lead can be added by other means and this invention is not limited to any particular method of adding the lead. In the experimental work which has been done it has been found that lead can be added to molten steel by using metallic lead, galena, an alloy of equal parts of lead, tin and antimony, a solder containing 60 per cent lead and 40 per cent tin, a bearing alloy containing 66 per cent copper, 32 per cent lead and 2 per cent tin, litharge and lead orthophosphate. It has been demonstrated that lead can be added to steel by all of the above as well as other lead-containing addition agents, and recoveries in the range of 15 to 64 per cent have been obtained. The recovery depends upon a number of factors. Increasing the holding time between the lead addition and pouring the steel seems to increase recovery of lead in the steel under some conditions. The recovery was better when relatively small additions, such as 0.40 per cent were made than when larger additions were made, such as 1.5 per cent. The chemical composition of the steel may have some influence on the recovery of lead but this relation has not been determined in a definite way. As will be shown hereinafter, lead has been added to steels of quite a range in chemical composition.

The solubility of lead in molten and in solid steel is not definitely known but a steel containing 0.53 per cent lead has been obtained with the indication that most, if not all, of the lead was in a state of dispersion instead of being in solution. It has been found that up to this amount, at least, the lead content continues to improve machinability.

Tests also show that, in cold drawing or lead-containing screw stock, the load required for reduction is diminished by 7.5 to 14.3 per cent for reductions in area of 1 to 21 per cent by a lead addition of .14 per cent and that the load is diminished by 10.2 to 19.6 per cent for similar reductions in area by a lead addition of .25 per cent. These cold drawn steels respectively contained, in addition to the lead content, .18 C, .81 Mn, .022 P, .134 S, .015 Si and .18 C, .75 Mn, .021 P, .127 S, .014 Si. Furthermore, commercial experience in machining steels made in accordance with my invention show that these steels containing lead remain much cooler than the so-called free cutting steels which is probably the result of less friction between the chip and the tool.

When lead is added in such amounts as 0.80 to 1.5 per cent it has been noted that there is a tendency for some of the lead to settle to the bottom of the containing vessel because of its high specific gravity. It is very probable, however, that by long holding and agitation at steel making temperature the lead contained in the steel can be materially increased above the value of 0.53 per cent which is the maximum that has been obtained so far in trial melts.

The addition of lead to relatively high sulfur steel of about 0.20 per cent sulfur and relatively low sulfur steel of about 0.03 per cent sulfur has also been studied and it appears that there is no essential difference in the amount of lead retained in the steel or in the relative amount recovered. It was found that the addition of lead to steels containing either a low percentage or a high percentage of sulfur definitely improved the machinability. When the lead is added in the form of galena there is an increase in the sulfur in the steel, due to the sulfur in the galena.

Lead has been added to steels of 0.80 and 1.35 per cent manganese contents and essentially the same recoveries and the same improvements in machinability obtained. Likewise, lead has been added to steels of 0.05 and 0.25 per cent silicon contents with no apparent differences in the amount of lead recovered or in its effect on machinability.

My researches have shown that the lead may be added at different stages in the production of the steel.

Lead in the various forms, such as metallic lead, lead sulfide and other compounds, has been added to the molten charge in an electric melting furnace of the high-frequency induction type. However, my preferred method of adding lead is:

To add it to the molten steel in the ingot mold in subdivided form after a small amount of steel has entered the mold by delivering a stream of sub-divided lead particles against the stream of steel pouring downwardly from the ladle and over a substantial period of time.

In studying the machinability of steels use has been made of saw and drill tests. A comparison has been made between the time required to saw a bar of cold rolled S. A. E. 1020 steel and experimental steel bars of the same size. From these data a "sawability index" has been calculated which is the time required to saw off a bar of the experimental steels divided by the time required for the standard bar of S. A. E. 1020. Similarly comparisons have been made in drilling tests in which the time required to drill to the same depth with all other conditions fixed in the standard S. A. E. 1020 steel, gives a "drillability index". It is evident that the smaller indices indicate better machinability. While many steels have been studied the following data will serve to show the advantages of lead in steels. The compositions of the steels and their indices are given in Table II.

TABLE II.—Effect of lead on machinability

| Steel No. | Chemical composition—percent |       |      |       |       |       | Machinability indices |          |
|-----------|------------------------------|-------|------|-------|-------|-------|-----------------------|----------|
|           | C                            | Si    | Mn   | P     | S     | Pb    | Sawing                | Drilling |
| 2962      | 0.11                         | 0.012 | 0.63 | 0.017 | 0.103 | Tr.   | .84                   | .98      |
| 2966      | 0.10                         | 0.012 | 0.55 | 0.019 | 0.204 | 0.122 | .69                   | .80      |
| 2967      | 0.11                         | 0.010 | 0.59 | 0.017 | 0.207 | 0.257 | .58                   | .73      |
| 2968      | 0.11                         | 0.010 | 0.58 | 0.019 | 0.214 | 0.342 | .53                   | .70      |
| 2969      | 0.11                         | 0.008 | 0.62 | 0.017 | 0.235 | 0.478 | .47                   | .69      |

It is obvious from the data in Table II that the machinability index is greatly improved by the addition of lead and that in the range covered, that is, from substantially more than traces to 0.478 per cent lead, the machinability improved as the lead content increased. It should be pointed out that steel No. 2962, in which the lead is present in traces only, is a relatively high-sulfur steel such as is now used in the trade as a free

cutting steel but as the lead content is increased the machinability is greatly improved.

Comparisons have been made of the machinability of the steels of this invention with commercial free cutting steels purchased in the open market. The results obtained on such commercial steel are shown in Table IIIA.

TABLE IIIA.—*Machinability tests on commercial free cutting steels*

| Steel No. | Description                      | Machinability indices |          |
|-----------|----------------------------------|-----------------------|----------|
|           |                                  | Sawing                | Drilling |
| 15        |                                  |                       |          |
| 1         | Commercial Bessemer.....         | .70                   | .96      |
| 2         | do.....                          | .77                   | .92      |
| 3         | do.....                          | .69                   | .92      |
| 4         | do.....                          | .70                   | .95      |
| 5-1       | Commercial open-hearth.....      | .88                   | .95      |
| 5-2       | Commercial Bessemer.....         | .71                   | .94      |
| 6         | do.....                          | .84                   | .94      |
| 7         | Commercial Bessemer X-grade..... | .72                   | .86      |

By comparing the data in Table IIIA with those in Table III it is evident that the steels of this invention containing 0.122 per cent or more lead have lower machinability indices and therefore have superior machinability. The superiority is most marked in the steels of higher lead content.

It is known that there are limitations to the improvement of the machinability of steels by the addition of increasing amounts of sulfur and other methods as now used in the art and one of the limitations is the loss of desirable properties in the finished product. The properties of the steels of this invention have been studied in many respects and it has been found that the addition of lead within the range of about .10 to .478 per cent has no significant harmful effect on the mechanical properties. This relation was determined by making tensile tests and Charpy impact tests on the steels listed in Table II, and it was found that by adding lead within the range shown in Table II the mechanical properties of yield strength, tensile strength, elongation and reduction of area were not materially changed by the addition of lead. Likewise, there was no significant change in the impact resistance when the lead was increased from a trace to 0.478 per cent. These tests were made on cold drawn bars and are therefore made on materials representative of commercial practice with free machining steels. It is evident that the addition of lead up to 0.478 per cent did not materially reduce any of these mechanical properties whereas the data in Table II show that such additions of lead greatly improved the machinability.

The effects of nitrogen and phosphorus additions have been studied. These elements are both hardening and strengthening in their function when added to steels. For that reason they may or may not improve machinability. If the steel is so soft that it has poor machinability then the addition of nitrogen or phosphorus or both of these elements tends to improve machinability. On the other hand, if the steel is sufficiently hard for good machinability then the addition of nitrogen or phosphorus or both of these elements may be detrimental to machinability because they increase the hardness to a value greater than the optimum for best machinability.

Using as a basis for comparison a low carbon steel of approximately .04 per cent carbon, .90 per cent manganese, .09 per cent silicon, .176 per cent sulfur, .012 per cent phosphorus and .008 per cent nitrogen, I have varied the nitrogen con-

tent up to .020 per cent, the phosphorus content up to .207 per cent and have added lead to this steel and then determined the hardness and tensile strength and the machinability as determined by sawing and drilling tests. Increasing the nitrogen as indicated above increased the hardness from 150 to 183 on the Brinell scale and the tensile strength from 71,000 to 81,500 p. s. i. Increasing the phosphorus as indicated above increased the hardness from 150 to 187 on the Brinell scale and the tensile strength from 71,000 to 91,000 p. s. i. Increasing the nitrogen as indicated above did not improve the machinability as determined by sawing tests and decreased it as determined by drilling tests. Increasing the phosphorus as indicated above only slightly improved the machinability as determined by sawing tests and materially decreased it as determined by drilling tests. On the other hand, when lead was added to the same base analysis in progressively increasing amounts, there was a proportionately definite improvement in machinability, as shown by both sawing and drilling tests. The addition of lead did not increase the hardness of hot rolled or cold drawn bars. Thus, it is evident that in practicing this invention it may be desirable in certain cases to vary the composition of the base steel to get the desired hardness and strength by adjusting the carbon, phosphorus, manganese, silicon and nitrogen. When the desired mechanical properties have been obtained lead is then added to improve machinability and the addition of lead has relatively little effect on the mechanical properties.

In the production of free cutting steels in accordance with my invention, the steels are preferably cold drawn to further improve the machinability thereof. This not only improves the machinability but facilitates the attainment of dimensional characteristics responding to the relatively close tolerances normally demanded by the industry.

As indicated above, my invention is directed mainly to steel. I am interested particularly in those ferrous alloys containing carbon in percentages less than 1.7 per cent. As stated above, my invention is applicable to any steel including high alloy steel which is intended for subsequent machining. My invention contemplates the use of lead in such steels in percentages ranging from 0.3 to 1 per cent. My invention also has especial utility in connection with the so-called "free cutting" steels wherein sulfur is present in percentages ranging from .05 to .30 per cent, since it has been found that the presence of lead there in in percentages ranging from .03 to 1 per cent markedly improves the free cutting characteristics of such steels.

With particular relation to free cutting steels of the character indicated, it will be seen that I have obtained highly important and novel results by the use of lead in proper quantities. As a matter of fact, I am able to produce a steel containing merely traces of sulfur or such quantities thereof as are unavoidable and, at the same time, to have such steel so freely machinable that it falls well within the class of free cutting steels, as far as adaptability for similar uses is concerned. Furthermore, the use of lead to obtain this enhanced machinability avoids all of the drawbacks which might result from the use of sulfur in relatively large quantities. In other words, the use of lead as a substitute for sulfur obtains the free machinability without any detrimental effects upon the physical properties of the steel.

It will also be understood that I may obtain the free machinability desired by the use of lead in a steel which also contains substantial quantities of sulfur. As the result of this, it is possible to obtain better results from the standpoint of machinability than hitherto possible where sulfur was mainly or entirely relied upon and without any sacrifice of the required or desired physical properties of the steel. As a matter of fact, by the use of lead either with or without sulfur, I have been able to produce a steel which is not only a free cutting steel but which will have physical properties superior to a steel of equal machinability wherein sulfur is mainly relied on to improve machinability.

The analyses given in Table III are the results of laboratory analyses of samples from the bars produced from the various melts and from the bars actually used in machinability tests. It will be observed that steel 3494 has no lead added while steel 3495 contained 0.07 per cent lead. The lead was added to these melts in the form of the oxide so that the sulfur content would not be increased by using galena. Likewise, for the remaining steels in Table III, one of each pair had no lead added while the other contained the amount shown.

The results of the mechanical tests on the heat treated bars are shown in Table IV.

TABLE IV.—Heat treatment and physical properties of experimental heats

| Heat No. | Pb      | Heat treatment                          | Yield strength* | Ultimate strength* | Elongation* | Reduction of area* | Charpy impact* | Brinell hardness | 20 |
|----------|---------|-----------------------------------------|-----------------|--------------------|-------------|--------------------|----------------|------------------|----|
|          | Percent |                                         | Lbs./sq. in.    | Lbs./sq. in.       | Percent     | Percent            | Ft./Lbs.       |                  |    |
| 3494     | 0.07    | 1600° F. 1 hr. air cooled.              | 44,900          | 62,250             | 40.0        | 66.5               | 50.0           | 114              |    |
| 3495     | do      | do                                      | 44,750          | 65,150             | 40.0        | 67.0               | 50.9           | 121              |    |
| 3496     | 0.187   | 1500° F. 1 hr. air cooled.              | 61,550          | 94,350             | 28.5        | 50.6               | 22.8           | 179              |    |
| 3497     | do      | do                                      | 64,750          | 97,900             | 28.5        | 52.0               | 23.8           | 170              | 10 |
| 3498     | 0.183   | 1450° F. 1 hr. air cooled.              |                 | 141,500            | 10.5        | 20.0               | 5.3            | 269              | 25 |
| 3499     | do      | do                                      |                 | 139,450            | 12.3        | 23.4               | 5.3            | 277              |    |
| 3502     | do      | 1500° F. 1 hr. furnace cooled.          |                 | 123,800            | 22.0        | 55.0               | 20.0           | 235              |    |
| 3503     | 0.158   | do                                      |                 | 147,800            | 17.5        | 44.9               | 15.0           | 262              |    |
| 3502     | do      | Oil Q. from 1500° F. D. 1000° F. 2 hrs. |                 |                    |             |                    |                | 341              | 30 |
| 3503     | 0.158   | do                                      |                 |                    |             |                    |                | 158              |    |
| 3569     | do      | Water Q. from 2000° F.                  |                 | 97,300             | 60.0        | 68.4               | 69.7           | 159              |    |
| 3570     | .08     | do                                      |                 | 98,000             | 57.0        | 66.7               | 68.0           | 159              |    |

\*Values shown are averages of duplicate tests.

Also, it will be seen that, by the use of lead to improve the machinability of the steel, I am also able to produce a steel which is more readily adaptable to hot-working. It may be hot-worked at lower temperatures without producing hot shortness in the steel, that is, without producing undue brittleness or lack of strength of the steel at red heat. In addition, this avoids the necessity for the prior art practice of increasing the manganese in the steel to offset the tendency towards hot shortness otherwise resulting from relatively large sulfur content. It will appear from this that a larger variety of free cutting steels can be produced where lead is mainly or entirely relied upon to obtain the desired free machinability.

Additional investigations that have been made show that lead can be used to improve the machinability of carbon steels of low to high carbon contents and of low to high alloy contents. Also, lead has been shown to improve the machinability of steels in the heat treated condition without loss in desired mechanical properties. Thus, steels of the analyses shown in the following Table III were cast, forged and rolled into one-inch bar stock which was then heat treated and tested for machinability by saw tests.

TABLE III.—Compositions of experimental heats of carbon and alloy steels

| Steel No. | Chemical composition—percent |      |      |      |      |      |      |      |       |
|-----------|------------------------------|------|------|------|------|------|------|------|-------|
|           | C                            | Mn   | Si   | P    | S    | Cr   | Ni   | Mo   | Pb    |
| 3494      | 0.15                         | 0.54 | 0.09 | .024 | .025 |      |      |      | None  |
| 3495      | 0.17                         | 0.85 | 0.11 | .025 | .025 |      |      |      | 0.07  |
| 3496      | 0.47                         | 0.74 | 0.09 | .027 | .025 |      |      |      | None  |
| 3497      | 0.46                         | 0.80 | 0.17 | .024 | .025 |      |      |      | 0.197 |
| 3498      | 0.88                         | 0.74 | 0.18 | .022 | .024 |      |      |      | 0.183 |
| 3499      | 0.88                         | 0.82 | 0.15 | .023 | .025 |      |      |      |       |
| 3502      | 0.48                         | 0.74 | 0.14 | .022 | .017 | 0.72 | 1.42 | 0.16 | 0.158 |
| 3503      | 0.49                         | 0.77 | 0.15 | .024 | .015 | 0.75 | 1.84 | 0.17 |       |
| 3569      | 0.14                         | 0.62 | 0.46 | .010 | .012 | 17.2 | 7.86 |      |       |
| 3570      | 0.14                         | 0.59 | 0.42 | .010 | .013 | 17.7 | 7.78 |      | 0.08  |

It is evident from Table IV that the addition of lead in the range of about 0.10 to about 0.20 per cent has not had a harmful effect on the mechanical properties of the steels.

Machinability tests have been made on these steels after heat treating the specimens with and without lead to give the comparison specimens approximately the same Brinell hardness. The results of my tests are shown in Table VIII.

TABLE V.—Effect of lead on sawability

| Steel No. | Car-<br>bon | Lead | Brinell<br>hard-<br>ness | Saw-<br>ability<br>index | Improve-<br>ment in<br>machin-<br>ability | Remarks         | 45 |
|-----------|-------------|------|--------------------------|--------------------------|-------------------------------------------|-----------------|----|
|           |             |      |                          |                          |                                           |                 | 50 |
| 3494      | .15         | .07  | 114                      | .93                      | 21                                        |                 |    |
| 3495      | .17         |      | 121                      | .73                      |                                           |                 |    |
| 3496      | .47         |      | 179                      | .68                      |                                           |                 |    |
| 3497      | .46         | .197 | 178                      | .51                      | 25                                        |                 |    |
| 3498      | .88         |      | 269                      | .72                      |                                           |                 |    |
| 3499      | .88         | .183 | 277                      | .56                      | 22                                        |                 |    |
| 3502      | .48         |      | 210                      | .64                      |                                           |                 |    |
| 3503      | .49         | .188 | 210                      | .55                      | 14                                        | Low alloy heat. | 55 |
| 3502      | .48         |      | 341                      | .73                      |                                           | Do.             |    |
| 3503      | .49         | .188 | 341                      | .58                      | 21                                        | Do.             |    |
| 3503      | .14         |      | 158                      | 1.55                     |                                           | 18-8 stainless. |    |
| 3569      | .14         | .08  | 159                      | 1.38                     | 11                                        | Do.             |    |
| 3570      |             |      |                          |                          |                                           |                 | 60 |

It is evident from the data in Table V that the addition of lead in every case improved the machinability, the improvement ranging from 11 per cent for the 18 per cent Cr-8 per cent Ni steel as quenched from 2000° F. to 25 per cent for the S. A. E. 1050 steel as normalized. The low alloy steel showed an improvement of 14 per cent when the hardness was higher (at 341 Brinell) the machinability was improved 21 per cent.

Tests have also been made on a high-manganese steel such as is known in industry as "austenitic manganese" steel or "Hadfield manganese" steel. This steel contained approximately 1.25 per cent carbon and 13-14 per cent man-

- ganese with no lead added to one heat and 0.50 per cent lead added to another. The rolled stock of these approximate analyses was heated to 1900° F. held for one hour and then quenched in water.
- 5 Machinists observed that the specimens to which the lead had been added machined more easily and produced a surface which showed less of what is known as "chatter" markings on the finished machined surface.
- 10 From the data cited earlier in this specification it is concluded that the machinability of the steels listed in Table III would have their machinabilities further improved by a larger addition of lead.
- 15 Ingots of leaded steel have been made in a commercial steel mill and commercial practice used in producing billets and bars. The analyses were of the low-carbon grade and the steels with and without the lead were essentially of the same analysis except steels E and F contained 0.10 per cent of lead. Mechanical tests showed that these steels had essentially the same yield and ultimate strength, the same elongation, reduction of area, Brinell hardness and Charpy impact resistance.
- 20 25 Machinability tests showed the following results:

| Steel No. | Lead     | Machinability index |       |          |
|-----------|----------|---------------------|-------|----------|
|           |          | Saw                 | Drill | Combined |
| 30        | Per cent |                     |       |          |
| E.....    | .10      | .66                 | .75   | .70      |
| F.....    | .10      | .68                 | .74   | .71      |
| G.....    | None.    | .85                 | .98   | .91      |

- 35 The method of making the machinability tests was the same as previously described and it is evident that the addition of 0.10 per cent lead materially improved the machinability.
- It will be understood that, in addition to free cutting steels and steels used for similar class of work, my invention is applicable to deep drawing steels, sheet steel, forging steels and carburizing steels in general of either straight carbon or alloy compositions.
- 45 My various tests are such as to indicate that the addition of lead in proper quantities to ingot irons and low-carbon steels that are "gummy" on machining, will also result in improved machinability of these irons which have hitherto been known to possess poor machinability. Thus it is indicated that such irons and steels as contain carbon in percentages from a trace to 0.10 per cent, from a trace to 0.20 per cent manganese, from a trace to 0.20 per cent phosphorus, from a trace to 0.20 per cent silicon and from a trace to .20 per cent sulfur, which normally have poor machinability, may have the machinability thereof greatly improved, even to the extent of giving them a machinability at least substantially equivalent to the normal free cutting steels, by the addition of .03 to 1.00 per cent of lead.
- It will be apparent from the above that my researches have so far shown that lead can be used to improve the machinability of carbon steels of low to high carbon contents and of alloy steels of low to high alloy contents. These researches indicate that steel containing such alloying elements as manganese, silicon, nickel, copper, chromium, molybdenum, vanadium, tungsten, zirconium, titanium, columbium, and tantalum may be improved by having incorporated therein variable percentages of lead.

Numerous other advantages of this invention will be apparent from the appended claims.

Having thus described my invention, what I claim is:

1. A steel consisting of carbon from effective amounts to 1.7 per cent, from .20 to 2.00 per cent manganese, from .01 to .20 per cent phosphorus, from .05 to .30 per cent sulfur, from .01 to 1.0 per cent silicon, from .03 to 1.0 per cent lead and the balance substantially all iron. 10
2. A steel consisting of carbon in percentages from effective amounts to 1.7 per cent, from traces to 2.0 per cent manganese, from traces to .20 per cent phosphorus, from traces to .30 per cent sulfur, from traces to 1.0 per cent silicon, 15 from .03 to 1.0 per cent lead, and the balance substantially all iron.
3. A ferrous alloy consisting of carbon in percentages from traces to 1.7 per cent, from traces to 2.0 per cent manganese, from traces to .20 per cent phosphorus, from traces to 0.5 per cent sulfur, from traces to 1.0 per cent silicon, from .03 to 1.0 per cent lead, the balance being substantially all iron. 20
4. A steel consisting of carbon in percentages from effective amounts to 1.7 per cent, from traces to 2.0 per cent manganese, from traces to .20 per cent phosphorus, from traces to .05 per cent sulfur, from traces to 1.0 per cent silicon, from .21 to 1.0 per cent lead and the balance substantially all iron. 25
5. A steel consisting of carbon in percentages from effective amounts to 1.7 per cent, from traces to 2.0 per cent manganese, from traces to .20 per cent phosphorus, from traces to .30 per cent sulfur, from traces to 1.0 per cent silicon, from .21 to 1.0 per cent lead and the balance substantially all iron. 30
6. A ferrous alloy consisting of carbon in percentages from traces to 1.7 per cent, from traces to 2.0 per cent manganese, from traces to .20 per cent phosphorus, from traces to 0.5 per cent sulfur, from traces to 1.0 per cent silicon, from .21 to 1.0 per cent lead, the balance being substantially all iron. 40
7. A steel containing carbon in effective amounts up to 1.7 per cent, sulfur in amounts from 0.05 to .50 per cent and lead in amounts from 0.1 to 0.478 per cent, the sulfur and lead cooperating to produce a free cutting steel, and the lead being substantially uniformly dispersed throughout the steel and having no significant harmful effect on its mechanical properties. 45
8. A steel containing carbon in effective amounts up to 1.7 per cent, sulfur in an amount less than 0.05 per cent, and lead in amounts from 0.1 to 0.478 per cent substantially uniformly dispersed throughout the steel and having no significant harmful effect on its mechanical properties, said steel having its machinability improved by the said lead. 50
9. A steel containing carbon in effective amounts up to 1.7 per cent and lead in amounts from 0.1 to 0.478 per cent, said lead being substantially uniformly dispersed throughout the steel and having no significant harmful effect on its mechanical properties, and said steel having its machinability so improved by the addition of lead that a sawability test shows an index better than that of otherwise identical steels containing substantially no lead. 55
- 70

OSCAR E. HARDER.

CERTIFICATE OF CORRECTION.

Patent No. 2,182,758.

December 5, 1939.

OSCAR E. HARDER.

It is hereby certified that error appears in the printed specification of the above numbered patent requiring correction as follows: Page 2, first column, line 23, beginning with "Dr. M. Hansen" strike out all to and including the word and period "steels." in line 18; and that the said Letters Patent should be read with this correction therein that the same may conform to the record of the case in the Patent Office.

Signed and sealed this 13th day of February, A. D. 1940.

(Seal)

Henry Van Arsdale,  
Acting Commissioner of Patents.